

3,365,329

PROCESS OF TREATING FABRICS TO RENDER  
THEM OIL- AND WATER-REPELLENT

Malcolm MacKenzie, Jr., Charlotte, and Roger James Martin, Jr., Greensboro, N.C., assignors to E. I. du Pont de Nemours and Company, Wilmington, Del., a corporation of Delaware

No Drawing. Filed June 30, 1964, Ser. No. 379,394  
2 Claims. (Cl. 117—161)

This invention is directed to an improvement in the process of treating fabrics to render them oil- and water-repellent and to provide significant repellencies that are durable to laundering and dry cleaning. More particularly, the present invention deals with the process of treating textile fabrics with (1) relatively small amounts of a fluoroalkyl-containing polymeric composition, (2) a composition comprising a wax and a stearic acid-hexamethylolmelamine derivative or a copolymer of (diethylamino)ethyl methacrylate and octadecyl methacrylate, and, optionally, (3) a crease resistant resin. In this novel process, a significant improvement is obtained by adding, to the dilute treatment bath containing these oil- and water-repellents, a dilute solution of a mixture of a selected anionic surface active agent of the sodium long chain alkyl sulfate or sulfated long chain alkenyl acetate types and a non-ionic surface active agent of a selected ethylene oxide condensation product. When the optional crease resistant resin is present in the treatment bath, only the selected anionic agent is added to obtain the improvement. The unexpected improvement provided by the invention mode of operation is a substantial increase in the initial oil- and/or water-repellency of the treated fabric and a high retention of these properties during repeated laundering and/or dry cleaning.

Oleophobic properties are commonly imparted to textile fabrics by treating them with selected polymeric polyfluoro materials. These compounds also impart water repellency. Water repellent effects are, however, commonly obtained with compositions comprising wax and a melamine derivative or a cationic polymeric material. These water repellent agents are often combined with the polyfluoro compositions to enhance the oil repellency and to provide a high water repellency in combination with the oil repellency. The increased oil repellency is advantageous, and the use of the lower cost wax-containing water repellent permits reducing the amount of the high cost polyfluoro material required for many applications. Crease resistant resins and other thermosetting resins which are employed, for example, to improve the hand of a fabric are frequently present in a textile treatment bath. These resins also enhance the repellent properties of fabric treated with fluorine-containing agents.

However effective the present combinations of agents are in rendering fabrics repellent (1) to oils and greases as vehicles and bonding agents for soils and (2) to water and water-borne liquid soils, there is room for improvement in keeping fabrics clean and unwetted and unaffected by water. Moreover, such oil- and water-repellent textile finishes need to be more durable to laundering and dry cleaning. The deposition on a fabric of lower amounts of the relatively expensive fluorine-containing oil repellent than are now commonly used to obtain a given effect would be both an economic advantage and a significant advance in the art.

It is, therefore, an object of this invention to improve the process of treating textile fibers to provide oil- and water-repellency. Another object is to enhance the oil- and water-repellency imparted to textile fibers by a combination of a polyfluoro polymeric oil-repellent and a selected wax composition for providing water-repellency. A further object is to increase the oil- and water-repel-

lency and the durability of these repellencies to laundering and dry cleaning when the repellencies are provided by compositions containing a relatively low amount of polyfluoro polymer.

5 These and other objects of the invention will become apparent from the following description and claims.

More specifically, the present invention is directed to the process of treating textile fabrics with (a) a fluoroalkyl-containing polymeric composition to impart oil- and water-repellency, and (b) a composition comprising a wax and a member of the group consisting of the acetic acid salt of a condensation product of hexamethylolmelamine, stearic acid, and triethanolamine and a copolymer of 2-(diethylamino)ethyl methacrylate and octadecyl methacrylate as a water repellent, the improvement being one which consists of adding to the dilute treatment bath, with agitation, a 5% to 15% aqueous solution of a mixture consisting of 60 to 75 parts by weight of a member of the group consisting of sodium C<sub>12</sub> to C<sub>16</sub> alkyl sulfates and the sodium salt of a sulfated C<sub>16</sub> to C<sub>18</sub> alkenyl acetate and 40 to 25 parts by weight of a condensation product of 10 to 20 moles of ethylene oxide and one mole of a member of the group consisting of C<sub>16</sub> to C<sub>18</sub> alkenyl alcohol and p-nonylphenol to provide from about 15% to about 30% by weight of said mixture on the basis of the said fluoroalkyl-containing polymeric composition and impregnating the fabric with the resultant treatment bath. A preferred embodiment is one wherein the treatment bath contains component (a) in an amount to give a pickup on the weight of the fabric from about 0.2% to about 0.5% of the component, and component (b) is present to the extent of 1 part to 5 parts per part of component (a).

35 The textile fabrics to which the present improved invention process may be applied include wool, cotton, acetate, nylon, polyacrylic fibers, polyester fibers, and their blends.

#### COMPONENTS OF TREATMENT BATH

40 (a) *Fluoroalkyl-containing polymeric composition.*— Such a composition is well known in the art for use in imparting oil-repellency and water-repellency to fabrics. The fluoroalkyl groups contained within the composition are perfluoroalkyl groups represented by C<sub>n</sub>F<sub>2n+1</sub> wherein n is an integer 4 to 14.

50 These groups form the terminal elements of various acrylate and methacrylate esters from which the polymeric material is made. These polymeric esters, copolymers of these esters and other polymerizable vinyl compounds, and mixtures of these copolymers and polymers or copolymers from polymerizable vinyl compounds are used as a water dispersion.

55 Specific, representative fluoroalkyl-containing polymeric compositions are the polymer, copolymer, and mixed polymer composition containing, as the principal fluorine-containing component,



60 wherein n is 4 to 14 as described in copending (common assignee) application Ser. No. 288,894, as well as Belgian Patent 634,720; French Patent 1,327,328 and Swiss Patent 5,274/62. Another group of fluoroalkyl-containing polymers and copolymers have, as the principal fluorine-containing component,



65 wherein n is 4 to 12, R is lower alkyl, R<sub>1</sub> is C<sub>1</sub> to C<sub>12</sub> alkylene and R<sub>2</sub> is hydrogen or methyl as described in U.S. Patent 2,803,615. The use of these fluorine-containing (a) polymers and copolymers with other materials is disclosed in French Patent 1,333,768.

(b) *Wax water-repellent composition.*—The defined composition of this component is well known in the art. It comprises 25% by weight of paraffin wax mixed with the acetic acid salt of the condensation product of hexamethylolmelamine, 2 moles stearic acid, and 1 mole triethanolamine, known in the trade as "Phobotex f/t/c" and described in U.S. Patent 2,783,231. In applying "Phobotex f/t/c," a catalyst consisting of a mixture of 70 parts by weight aluminum glycolate and 30 parts by weight of glycolic acid is employed in an amount equal to 10% by weight of the "Phobotex f/t/c" to achieve maximum durability of this particular water-repellent textile finish.

The composition also comprises a dispersion of a mixture of a copolymer of (diethylamino)ethyl methacrylate and octadecyl methacrylate and paraffin wax as described in Example 4 of British Patent 915,759 using 30 parts of the basic monomer to form the comonomer and a wax:copolymer ratio of 3:1.

(c) *Crease resistant resin.*—This optional component of the treatment bath is a thermosetting resin frequently employed to impart crease resistance to a fabric. The resins of this type which may be added to the treatment bath include commercially available urea-formaldehyde resins, melamine-formaldehyde and methylol derivatives of cyclic ethylene ureas, triazone derivatives, and urons. The use of these resins is accompanied by catalysts designed for the fixation of the resins. The catalysts include amine hydrochlorides, metal salts such as magnesium chloride and zinc nitrate.

When a crease resistant resin is present in the treatment bath only the anionic agent is added in an amount equal to about 2% to 10% of the fluoroalkyl composition.

The relative amounts of the fluoroalkyl-containing polymeric composition and the wax water-repellent composition in the textile finishing bath affect the degree of oil- and water-repellency obtained. For the best results the proportion of these components will vary with different fabrics and conditions of application. In general, a minimum of 0.2% by weight of the fluoropolymer composition on the weight of the fabric is needed, and more than 0.65% by weight is considered uneconomical. The preferred amounts are within the range of 0.25% to 0.45%. The amount of the wax-containing water-repellent composition should be adjusted to fall within the range of 1 part to 5 parts per part of the fluoropolymer composition. When the ratio of the wax-containing water-repellent to the fluoropolymer composition is much higher than 5:1, the oil repellency is decreased. If the ratio of these components is much less than 1:1, there is a deficiency of the water-repellent component and the water repellency of the finished fabric is decreased.

The crease resistant resin, when applied together with the oil- and water-repellents, is deposited to the extent of 1% to 5% by weight on the weight of the fabric. Within this range the ratio of the resin to the fluoropolymer composition is not critical.

#### ADDED SURFACE ACTIVE AGENTS

The anionic surface active agents of particular value in practicing this invention are sodium  $C_{12}$  to  $C_{16}$  alkyl sulfates and the sodium salt of a sulfated  $C_{16}$  to  $C_{18}$  alkenyl acetate. These dispersing agents are usually employed in combination with non-ionic surfactants, although they are effective when used alone in a pad bath containing a crease resistant resin in combination with the oil- and water-repellents. The non-ionic surface active agents that are blended with the anionic agents are the condensation product of 10 to 20 moles of ethylene oxide with 1 mole of technical oleyl alcohol ( $C_{16}$  to  $C_{18}$  alkenyl alcohol) and the product of 9 to 10 moles of ethylene oxide condensed with 1 mole of p-nonylphenol. The mixture of surface active agents consists of 60 to 75 parts by weight of the anionic agent and 40 to 25 parts by weight of the non-ionic agent. The mixture is added to the

treatment bath as a water solution of 5% to 15% concentration to provide from about 15% to about 30% by weight of the mixture of agents on the basis of the fluoroalkyl-containing polymeric composition. When added singly to a treatment bath containing a crease resistant resin a dilute solution of the anionic surfactant of 5% to 15% concentration provides from 2% to 10% by weight of the fluoroalkyl polymer of the anionic additive.

It is unexpected that the addition to the treatment bath of limited amounts of selected anionic agents, used alone or in combination with certain non-ionic surface active agents, makes possible the marked improvement in the oil- and water-repellency and in the durability of these repellencies. These favorable results are particularly surprising because many of the materials normally present in the treatment bath are cationic or are salts of metals which would be expected to be incompatible with water-soluble anionic agents. For instance, many of the fluoropolymer composition dispersions are cationic; so are the wax water-repellent dispersions. The catalysts used in various composites of textile treating agents in the invention process contribute polyvalent metal ions which have an insolubilizing action on anionic surfactants. Heretofore, those skilled in the art of finishing textile fabrics have taken pains to avoid any contamination from anionic surface active agents in the treatment bath. Excessive amounts of the anionic surfactants of the invention process do cause coagulation of the dispersed materials in the treatment bath, but the controlled amounts employed in the manner described give improved finishes on the goods treated according to the invention.

#### GENERAL PROCEDURE

The practice of this invention, in its simplest form, involves the padding of a fabric in a bath containing the fluoropolymer dispersion together with a dispersed wax-containing water-repellent composition, its catalyst if needed, and the selected surfactant adjuvants. When the wax-containing water-repellent composition is "Phobotex f/t/c," two parts of hot water are mixed with stirring with one part of the water-repellent and heated to the boil to melt the solid material. One-tenth part of the aluminum glycolate-glycolic acid catalyst, is added and the stirring continued to complete the emulsification. The concentrated emulsion is diluted with water at about 38° C. to give 75% of the ultimate volume. The fluoropolymer dispersion is then added with agitation followed by the surfactant adjuvants as a 10% water solution. The bath is adjusted to its final volume with water and is ready for use in the normal manner.

When a crease resistant resin is present in the treatment bath, it is customary to use the anionic surfactant adjuvant alone. In this case, the wax-containing water-repellent composition is emulsified as described above, the emulsion is diluted with water at about 38° C. and the anionic adjuvant is added as a 10% water solution with efficient agitation. The crease resistant resin and its catalyst are added followed by the fluoropolymer dispersion to obtain a bath ready for use.

The treatment bath is used at a temperature within the range of 20° C. to 35° C. in a 2- or 3-roll padder of the type normally employed in applying resins to fabrics. A weight pickup of 40% to 100% is attained, and the concentration of the components of the bath are adjusted accordingly to give the desired dry weight pickup on the weight of the fabric. After padding, the fabric is dried under conditions that are not critical. Frame drying is preferred to can or roller drying to avoid possible transfer of the finishing agents to the can or roller. A curing or heating step follows. The conditions of cure depend upon the heat stability of the textile fiber and the requirements for developing the best repellency and fastness (to laundering and dry cleaning) properties. Curing times and temperature will also vary with fabric weight and with different pieces of equipment. Usually

1 minute to 3 minutes at from 150° C. to 175° C. are taken for curing.

While the invention process finishes are usually applied by padding, they may also be applied by spraying or other means by which a textile fabric is impregnated with a treatment bath of finishing materials.

### TESTING OF FABRICS

The treated fabric samples are tested for water repellency by the Standard Test Method 22-1961 of the American Association of Textile Chemists and Colorists. A rating of 100 denotes no water penetration or surface adhesion, a rating of 90 denotes slight random wetting and so on.

The oil repellency test comprises placing a drop of test oil carefully on the textile on a flat horizontal surface. After ten seconds any penetration or wicking into the fabric is noted visually. The nature of the test oil and the respective oil repellency ratings are:

| Test solution:           | Oil repellency rating |
|--------------------------|-----------------------|
| n-Heptane                | 9                     |
| n-Octane                 | 8                     |
| n-Decane                 | 7                     |
| n-Dodecane               | 6                     |
| n-Tetradecane            | 5                     |
| 50/50 hexadecane/"Nujol" | 4                     |
| 25/75 hexadecane/"Nujol" | 3                     |
| "Nujol"                  | 2                     |
| "Nujol" wets             | 0                     |

In assigning a rating, for example, if a treated fabric repels the number 1 to 6 solutions but not number 7, its rating is 6.

After obtaining the initial oil- and water-repellency ratings of the fabric specimens, portions of them are subjected to three standard launderings and three standard dry cleanings as a test of the durability of the finish. The laundering test is carried out in a machine described in Federal Specification CCC-T191b, Method 5550. Soft water is added to the machine to a depth of 5 to 7 inches, and with fabrics of cotton, polyester fibers, and their blends the water is heated to the boil. For other fabrics such as wool, nylon, acetate and their blends, the water is heated to 50° C. Neutral soap in a concentration of 0.1% based on the weight of water in the machine is added, and, in the case of cotton or polyester fibers, 0.05% soda ash is also added. Test specimens of fabric together with other fabric specimens to give a total dry load of three pounds are placed in the machine. The fabrics are subjected to washing action for 40 minutes when they are removed, rinsed, and squeezed flat. A fabric specimen is dried on a at press at about 150° C. for 30 seconds on each side. It is conditioned at 20° C. and 65% relative humidity for at least 4 hours before making repellency tests. The dry cleaning test is conducted in an American Association of Textile Chemists and Colorists' Standard Launder-Ometer. A specimen, 20 cm. x 25.4 cm., is placed in a 500 ml. jar with 150 ml. of tetrachloroethylene, 2.25 g. of a commercial dry cleaning detergent, and 0.15 g. of water. The jar is placed in the Launder-Ometer and tumbled for 20 minutes at 27° C. Excess solvent is removed by blotting between blot-

ting paper, and the fabric is air-dried, then dried for 15 seconds on each side on a flat press at about 150° C., and ironed. The dry-cleaned specimen is conditioned at least four hours at 20° C. and 65% relative humidity before testing for repellency.

In order to assure good stain and soil resistant performance of fabric in service, it is customary to require a degree of repellency that has been found from experience to be satisfactory in terms of the results of oil-repellency and water repellency tests. Fabrics destined for use in rainwear and outerwear are required to have a minimum spray test rating of 90 initially and 80 after three standards launderings or three standard dry cleanings as described above. The oil repellency requirement is a minimum rating of 6 initially and 5 after three standard launderings or dry cleanings. Fabrics designed for general apparel, draperies, and slipcovers require a minimum spray test rating initially of 80 and 70 after three standard launderings or dry cleanings. The oil repellency rating on these fabrics should be a minimum of 5 initially and of 4 after the three launderings or dry cleanings.

Representative examples further illustrating the invention follow:

#### Example 1

A sample of cotton wide wale corduroy was padded to a wet pickup of 100% with a treatment bath containing 0.46% of a mixture of copolymers consisting of 40 parts of—

|    |                                                                                                                                                                |
|----|----------------------------------------------------------------------------------------------------------------------------------------------------------------|
| 30 | (A) Copolymer of:                                                                                                                                              |
| 35 | (1) $F(CF_2)_nCH_2CH_2O_2C(CH_3)C=CH_2$<br>wherein $n$ is 6, 8, and 10 in the ratio of 3:2:1<br>with small amounts of monomer with $n=12$<br>and 14 ----- 97.5 |
| 35 | (2) Butyl acrylate ----- 2.0                                                                                                                                   |
| 35 | (3) N-methylolacrylamide ----- 0.5                                                                                                                             |

and 60 parts of—

|    |                                       |
|----|---------------------------------------|
| 40 | (B) Copolymer of:                     |
| 45 | (1) 2-ethylhexylmethacrylate ----- 98 |
| 45 | (2) N-methylolacrylamide ----- 2      |

45 The 0.46% of the mixed copolymers was obtained from using 3.5% of a 13% dispersion of the copolymer mixture stabilized with the acetic acid salt of dimethyloctadecylamine. The bath also contained 1% of the acetic acid salt of a condensation product of hexamethyolmelamine, 50 stearic acid, and triethanolamine mixed with 0.33 part of paraffin wax per part of condensation product salt ("Phobotex f/t/c" water repellent supplied by the Ciba Company) and 0.1% of the acidic aluminum glycolate catalyst. The fabric was dried for 5 min. at 120° C. then 55 heated 2 min. at 170° C. (control specimen). Another sample of the corduroy was similarly treated with a pad bath the same as above with 0.11% by weight of a mixture containing 73% by weight of the sodium salt of sulfated C<sub>16</sub>-C<sub>18</sub> alkenyl acetate and 27% by weight of the condensation product of 10 moles of ethylene oxide and 1 mole of technical oleyl alcohol (exhibit specimen).

The initial water repellency (spray rating) and oil repellency and the durability of these repellencies after three standard launderings and dry cleanings as described above are as follows:

| Fabric       | Water Repellency |                     |                       | Oil Repellency |                     |                       |
|--------------|------------------|---------------------|-----------------------|----------------|---------------------|-----------------------|
|              | Initial          | After 3 Launderings | After 3 Dry Cleanings | Initial        | After 3 Launderings | After 3 Dry Cleanings |
| Control----- | 100              | 90                  | 80                    | 5              | 4                   | 0                     |
| Exhibit----- | 100              | 100                 | 80                    | 7              | 7                   | 6                     |

The significant improvement in the finish of this fabric provided by the surfactant adjuvants is the increased initial oil repellency, its retention during repeated launderings and dry cleaning, and the retention of the water repellency during laundering.

*Example 2*

A sample of wool flannel was padded to a wet pickup of 75% with a treatment bath containing 0.65% by weight of the fluoroalkyl-containing copolymer mixture of Example 1 and 0.8% of "Phobotex f/t/c" water repellent with 0.08% catalyst. The fabric was air-dried then heated 7.5 minutes at 150° C. (control specimen). Another sample of the wool flannel was similarly padded with a bath the same as above except that 0.169% by weight of a mixture containing 75% by weight of the sodium salt of sulfated C<sub>16</sub>-C<sub>18</sub> alkenyl acetate and 33% by weight of the condensation product of 10 moles of ethylene oxide and 1 mole of p-nonylphenol was added (exhibit specimen). The initial water repellency and oil repellency and the durability of these repellencies after three standard dry cleanings are as follows:

| Fabric       | Water Repellency |                       | Oil Repellency |                       |
|--------------|------------------|-----------------------|----------------|-----------------------|
|              | Initial          | After 3 Dry Cleanings | Initial        | After 3 Dry Cleanings |
| Control..... | 90 to 100        | ( <sup>1</sup> ) 80   | 0              | 0                     |
| Exhibit..... | 100              | 80                    | 7              | 7                     |

<sup>1</sup> No data.

A high oil repellency is imparted to the fabric which without the invention treatment is devoid of this property, and the finish survives repeated dry cleanings.

When the foregoing treatment was repeated with wool gabardine with the employment of the condensation product of 10 moles of ethylene oxide and 1 mole of technical oleyl alcohol in place of the ethylene oxide/p-nonylphenol condensation product for the exhibit sample the same results were obtained.

With wool flannel the treatment as first given in the example was repeated replacing 0.8% of the "Phobotex f/t/c" water-repellent with 6% of a 28% by weight dispersion of the wax/copolymer composition of Example 4 of British Patent 915,759 wherein the copolymer was prepared from 30 parts by weight of 2-(diethylamino)ethyl methacrylate and 70 parts by weight of octadecyl methacrylate and the ratio of wax to copolymer was 3 to 1. The initial water and oil repellencies are as follows:

| Fabric       | Water Repellency | Oil Repellency |
|--------------|------------------|----------------|
| Control..... | 80               | 2              |
| Exhibit..... | 90               | 5              |

A significant improvement in the repellency of both water and oil is obtained.

*Example 3*

A 55/45 polyester fiber/wool suiting fabric was padded at 27° C. to a wet pickup of 75% with a treatment bath containing 0.52% by weight of the fluoroalkyl-containing copolymer mixture of Example 1 and 1.0% of "Phobotex f/t/c" water repellent with the usual 0.1% of catalyst for this water repellent. The fabric was dried at about 90° C. and heated for five minutes at 145° C. (control specimen). Another sample of the fabric was given the same treatment except that now the pad bath contained in addition to the oil and water repellency agents, 0.127% by weight of a mixture containing 74% by weight of the sodium salt of sulfated C<sub>16</sub>-C<sub>18</sub> alkenyl acetate and 26% by weight of the condensation product of ethylene oxide and technical oleyl alcohol used in Example 1 (exhibit specimen). The initial water repellency and oil repellency and the

durability of these repellencies after three standard dry cleanings are as follows:

| Fabric       | Water Repellency |                       | Oil Repellency |                       |
|--------------|------------------|-----------------------|----------------|-----------------------|
|              | Initial          | After 3 Dry Cleanings | Initial        | After 3 Dry Cleanings |
| Control..... | 90               | 0                     | 4              | 0                     |
| Exhibit..... | 100              | 80                    | 7              | 4                     |

A definite increase in the initial water repellency, a marked improvement in the oil repellency, and a high retention compared to a complete loss of these properties during repeated dry cleanings are to be noted.

When the foregoing treatment was given to specimens of a 55/45 polyester fiber/cotton fabric the following results were obtained:

| Fabric       | Water Repellency |                       | Oil Repellency |                       |
|--------------|------------------|-----------------------|----------------|-----------------------|
|              | Initial          | After 3 Dry Cleanings | Initial        | After 3 Dry Cleanings |
| Control..... | 90               | 0                     | 4              | 0                     |
| Exhibit..... | 100              | 50                    | 7              | 4                     |

A particularly significant improvement is the higher initial oil repellency and a retention of this property during dry cleaning.

*Example 4*

An acetate velvet fabric was padded at 27° C. to a wet pickup of 100% with a treatment bath containing by weight

|                                                                | Percent |
|----------------------------------------------------------------|---------|
| Fluoroalkyl-containing copolymer mixture of Example 1          | 0.33    |
| "Phobotex f/t/c" water repellent                               | 0.8     |
| Catalyst                                                       | 0.08    |
| Tartaric acid                                                  | 0.025   |
| Ethylene oxide/p-nonylphenol condensation product of Example 2 | 0.05    |

The fabric was dried at 135° C. and heated ten minutes at 160° C. (control fabric). A second portion of the fabric was treated in the same way with 0.076% by weight of a mixture of the anionic and nonionic surfactants of Example 3 added to the padding bath (exhibit fabric). The repellency tests of these treated fabric specimens are as follows:

| Fabric       | Water Repellency |                       | Oil Repellency |                       |
|--------------|------------------|-----------------------|----------------|-----------------------|
|              | Initial          | After 3 Dry Cleanings | Initial        | After 3 Dry Cleanings |
| Control..... | 80               | 50                    | 4              | 3                     |
| Exhibit..... | 100              | 80                    | 6              | 4                     |

A significant improvement in both the water and oil repellency is achieved, and these properties resist dry cleaning.

*Example 5*

A wool suiting fabric was padded at 32° C. to a wet pickup of 65% with a treatment bath containing 0.75% by weight of the fluoroalkyl-containing copolymer mixture of Example 1 and 0.92% of "Phobotex f/t/c" water repellent with 0.09% catalyst. The fabric was dried and cured 7.5 minutes at 150° C. (control). A second portion of the fabric was treated in the same way except the bath contained an added component amounting to 0.17% by weight of the bath of a mixture of 75% sodium dodecyl sulfate and 25% of the ethylene oxide/technical oleyl alcohol condensation product of Example 1 (exhibit spec-

imen). The repellency tests of these treated fabric specimens are as follows:

| Fabric       | Water Repellency |                       | Oil Repellency |                       |
|--------------|------------------|-----------------------|----------------|-----------------------|
|              | Initial          | After 3 Dry Cleanings | Initial        | After 3 Dry Cleanings |
| Control----- | 80               | 70                    | 4              | 2                     |
| Exhibit----- | 100              | 80                    | 5              | 4                     |

An enchantment of the initial water and oil repellency and improvement in retention of the oil repellency during repeated dry cleaning by the addition to the treatment bath of the mixture of surfactants are apparent.

*Example 6*

A wool suiting fabric was padded at 32° C. to a wet pickup of 75% with a treatment bath containing 0.84% by weight of a copolymer of 50/50 2(N-propylhepta-deafluoroctylsulfonamido)ethyl acrylate/chloroprene. This fluoroalkyl-containing copolymer mixture was added to the bath as a 28% water dispersion as described in U.S.P. 2,803,615. The treatment bath also contained 0.8% by weight of "Phobotex f/t/c" water repellent with 0.08% catalyst. The fabric was then dried and cured 7.5 minutes at 150° C. (control). A second portion of the fabric was treated in the same way but with 0.14% by weight of a mixture of 75% sodium dodecyl sulfate and 25% of the ethylene oxide/technical oleyl alcohol condensation product of Example 1 added to the treatment bath (Exhibit A). A third portion of the same fabric was treated like Exhibit A with sodium hexadecyl sulfate employed as the anionic component of the added surfactant mixture (Exhibit B). The following repellency test results were obtained:

| Fabric         | Water Repellency |                       | Oil Repellency |                       |
|----------------|------------------|-----------------------|----------------|-----------------------|
|                | Initial          | After 3 Dry Cleanings | Initial        | After 3 Dry Cleanings |
| Control-----   | 80               | 70                    | 4              | 3                     |
| Exhibit A----- | 100              | 80                    | 6              | 4                     |
| Exhibit B----- | 100              | 80                    | 6              | 4                     |

In each case the addition to the treatment bath of the

The fabric was padded to a 100% pickup, dried at 135° C., and heated 1.5 minutes at 163° C. followed by a mild alkaline wash and ironing at 150° C. (exhibit specimen). A control specimen was prepared by the same procedure except the sodium sulfated alkenyl acetate was omitted from the pad bath. The fabric specimens were tested for initial water and oil repellency and for retention of the oil repellency during three dry cleanings with the results shown below:

| Fabric       | Water Repellency<br>After<br>3 Dry<br>Cleanings | Oil Repellency |                             |
|--------------|-------------------------------------------------|----------------|-----------------------------|
|              |                                                 | Initial        | After<br>3 Dry<br>Cleanings |
| Control----- | 0                                               | 6              | 2                           |
| Exhibit----- | 80                                              | 7              | 6                           |

The marked effect of the addition of the anionic agent to the pad bath on the durability to repeated dry cleaning of the water and oil repellency is apparent.

*Example 8*

A textile finishing pad bath was prepared to contain:

|                                                                                 | Percent |
|---------------------------------------------------------------------------------|---------|
| Fluoroalkyl - containing copolymer mixture of                                   |         |
| Ex. 1 -----                                                                     | 0.39    |
| "Phobotex f/t/c" water repellent -----                                          | 1.20    |
| Catalyst -----                                                                  | 0.12    |
| Modified triazine crease resistant resin ("Aerotex 23" American Cyanamid) ----- | 1.5     |
| Magnesium chloride -----                                                        | 0.24    |
| Tartaric acid -----                                                             | 0.025   |
| Isopropyl alcohol -----                                                         | 5.0     |
| Sodium salt of sulfated C <sub>16</sub> -C <sub>18</sub> alkenyl acetate -----  | 0.033   |

Cotton rainwear fabric was padded at 30° C. to 100% pickup in the above bath, dried at 135° C., and heated 2.5 minutes at 170° C. The cured fabric was then washed in a bath at 50° C. containing 0.1% soda ash and 0.05% sodium dodecyl sulfate, followed by rinsing at 50° C. and ironing at 150° C. (exhibit specimen). A control specimen was prepared by the same procedure except the sodium sulfated alkenyl acetate was omitted from the pad bath. The fabrics were tested with the results shown below:

| Fabric       | Water Repellency |                     |                       | Oil Repellency |                     |                       |
|--------------|------------------|---------------------|-----------------------|----------------|---------------------|-----------------------|
|              | Initial          | After 3 Launderings | After 3 Dry Cleanings | Initial        | After 3 Launderings | After 3 Dry Cleanings |
| Control----- | 100              | 70                  | 70                    | 7              | 5                   | 7                     |
| Exhibit----- | 100              | 90                  | 90                    | 7              | 7                   | 7                     |

mixture of the anionic and the non-ionic surface active agents has effected an improvement in the initial water and oil repellency. The retention of these properties during repeated dry cleanings relative to the control is little changed.

*Example 7*

An aqueous treatment bath for padding a fabric consisting of a 65/35 blend of polyester fiber/cotton contained the following finishing agents:

|                                                                                 | Percent |
|---------------------------------------------------------------------------------|---------|
| Fluoroalkyl-containing polymer mixture of Exam-<br>ple 1 -----                  | 65      |
| "Phobotex f/t/c" water repellent -----                                          | 0.52    |
| Catalyst -----                                                                  | 1.0     |
| Modified triazine crease resistant resin ("Aerotex 23" American Cyanamid) ----- | 0.1     |
| Melamine formaldehyde crease resistant resin<br>(Resin M-3) -----               | 3.6     |
| Zinc nitrate -----                                                              | 1.7     |
| Sodium salt of sulfated C <sub>16</sub> -C <sub>18</sub> alkenyl acetate -----  | 0.64    |

Significant effects of the added surface active agent are the increased retention of water repellency during repeated laundering and repeated dry cleaning and of oil repellency during repeated laundering.

*Example 9*

A textile finishing pad bath consisting of:

|                                                                                | Percent |
|--------------------------------------------------------------------------------|---------|
| Fluoroalkyl-containing copolymer mixture of                                    |         |
| Ex. 1 -----                                                                    | 0.32    |
| "Phobotex f/t/c" water repellent -----                                         | 1.0     |
| Catalyst -----                                                                 | 0.1     |
| Urea-formaldehyde crease resistant resin -----                                 | 70 4.0  |
| Magnesium chloride -----                                                       | 0.25    |
| Tartaric acid -----                                                            | 0.06    |
| Isopropyl alcohol -----                                                        | 2.0     |
| Sodium salt of sulfated C <sub>16</sub> -C <sub>18</sub> alkenyl acetate ----- | 0.007   |
| Water to make -----                                                            | 100.00  |

11

Cotton print fabric was padded at 33° C. to 100% pickup in the above bath, dried at 135° C., and heated three minutes at 170° C. Another portion of the fabric was similarly padded without the sodium sulfated alkenyl acetate in the pad bath and dried and cured in the same way to provide a control specimen. The results of repellency tests on the two fabric specimens are as follows:

| Fabric       | Water Repellency |                     |                       | Oil Repellency |                     |                       |
|--------------|------------------|---------------------|-----------------------|----------------|---------------------|-----------------------|
|              | Initial          | After 3 Launderings | After 3 Dry Cleanings | Initial        | After 3 Launderings | After 3 Dry Cleanings |
| Control..... | 80               | 70                  | 50                    | 8              | 5                   | 0                     |
| Exhibit..... | 80               | 80                  | 70                    | 7              | 5                   | 7                     |

In the above treatment the added anionic agent has definitely increased the durability of the water repellency to repeated laundering and dry cleaning and markedly improved oil-repellency finish for resisting repeated dry cleaning.

The preceding representative examples may be varied within the scope of the present total specification disclosure, as understood and practiced by one skilled in the art, to achieve essentially the same results.

As many apparently widely different embodiments of this invention may be made without departing from the spirit and scope thereof, it is to be understood that this invention is not limited to the specific embodiments thereof except as defined in the appended claims.

The embodiments of the invention in which an exclusive property or privilege is claimed are as follows.

We claim:

1. In the process of treating textile fabric with a dilute treatment bath comprising (a) a fluoroalkyl-containing polymeric composition to impart oil- and water-repellency, and (b) a composition comprising (1) a wax and a member of the group consisting of (2) the acetic acid salt of a condensation product of hexamethylolmelamine, stearic acid, and triethanolamine and (3) a copolymer of 2-(diethylamino)ethyl methacrylate and octadecyl methacrylate as a water repellent, the improvement which con-

sists of adding to the dilute treatment bath, with agitation, a 5% to 15% aqueous solution of a mixture consisting of (A) 60 to 75 parts by weight of a member of the group consisting of (I) sodium C<sub>12</sub> to C<sub>18</sub> alkyl sulfates and (II) the sodium salt of a sulfated C<sub>16</sub> to C<sub>18</sub> alkenyl acetate and (B) 40 to 25 parts by weight of a condensation product of 10 to 20 moles of ethylene oxide and 1 mole of a

12

member of the group consisting of C<sub>16</sub> to C<sub>18</sub> alkenyl alcohol and p-nonylphenol to provide from about 15% to about 30% by weight of said mixture on the basis of said fluoroalkyl-containing polymeric composition and impregnating the fabric with the resultant treatment bath.

2. A process according to claim 1 wherein the treatment bath contains said component (a) in an amount to give a pickup on the weight of the fabric from about 0.2% to about 0.5% of the component, and said component (b) is present to the extent of 1 part to 5 parts per part of said component (a).

#### References Cited

##### UNITED STATES PATENTS

- |           |         |                                |
|-----------|---------|--------------------------------|
| 2,803,615 | 8/1957  | Ahlbrecht et al.               |
| 3,256,231 | 6/1966  | Johnson et al. ----- 260—900   |
| 3,277,039 | 10/1966 | Marascia et al. ----- 260—29.6 |
| 3,282,905 | 11/1966 | Fasick ----- 260—29.6          |

##### FOREIGN PATENTS

- |           |        |                |
|-----------|--------|----------------|
| 915,759   | 1/1963 | Great Britain. |
| 1,333,768 | 6/1963 | France.        |

WILLIAM D. MARTIN, *Primary Examiner.*

T. G. DAVIS, *Assistant Examiner.*